

Dec. 7, 1954

A. F. KRITSCHER

2,696,378

METHOD OF HEATING STEEL SLUGS FOR FORGING OR EXTRUSION

Filed Aug. 13, 1951

FIG. 1.



FIG. 2.



FIG. 3.



FIG. 4.



FIG. 5.



FIG. 6.



FIG. 8.



FIG. 7.



Inventor:

ANDREW F. KRITSCHER,  
by: Donald G. Dalton  
his Attorney.

## METHOD OF HEATING STEEL SLUGS FOR FORGING OR EXTRUSION

Andrew F. Kritscher, Mount Lebanon Township, Allegheny County, Pa., assignor to United States Steel Corporation, a corporation of New Jersey

Application August 13, 1951, Serial No. 241,619

7 Claims. (Cl. 263—52)

This invention relates to the heating of masses of metal and, in particular, to the heating of billets or slugs of steel for hot-working by extrusion or forging.

The extrusion of steel through forming dies has been accomplished but requires a special technique and is still beset with numerous difficulties. For example, the heating of the billets or slugs has usually been effected in conventional furnaces at relatively low rates. The heavy scale resulting is abrasive in character and causes rapid wear of the dies, besides reducing the product yield per pound of billet weight. Such scale is not fully removed by conventional descaling practice and the portion left on the billets impairs the surface finish of the extruded product, besides damaging the dies. In addition, the power required for the extrusion operation has been very high. Experience has shown, furthermore, that stainless-steel billets heated by conventional methods and equipment, i. e., involving long heating times such as several hours, occasionally will not "push" when placed in the press, although heated to the proper temperature.

I have invented a novel method of heating steel billets or slugs for extrusion which overcomes these difficulties and is characterized by further important advantages. The invention is also useful in heating billets for ordinary forging operations. My invention is based on the fact that ordinary steel, while losing most of its tensile strength at temperatures in the neighborhood of those required for forging or extrusion, still retains sufficient strength at such temperatures to sustain substantial loads. Recent investigations show, for example, that low-carbon steel has a short-time tensile strength of about 2500 p. s. i. at 2000° F. and about 1500 p. s. i. at 2300° F. I take advantage of this fact to provide a novel method of supporting and handling billets or slugs while being heated for working by forging or extrusion. I also utilize an improved type of heating furnace and effect the heating at a rate much greater than has been thought possible heretofore. I am thereby enabled to utilize fully the short-time strength at high temperatures.

In a preferred practice, I weld a steel stud to one end of a billet or slug and, by means of the welded-on stud, I support the slug while conveying it through a continuous, panel-type furnace which heats it rapidly to extrusion or forging temperature. After the billet has been heated and while still suspended by the stud, I subject it on emerging from the furnace to a descaling treatment and also immerse it in a fused salt bath heated to about the desired final temperature of the billet. After a short time, I remove the billet from the bath, shear off the stud and then deliver the billet immediately to the extrusion press.

A complete understanding of the invention may be obtained from the following detailed description and explanation which refer to the accompanying drawings illustrating the present preferred practice. In the drawings,

Figure 1 is a diagrammatic elevation illustrating the welding of a stud to one end of a billet;

Figure 2 is an elevation partly broken away showing the heating furnace with a billet traveling therethrough;

Figure 3 is a partial cross-section through the furnace;

Figure 4 is a vertical section through a water-spray descaler;

Figure 5 is a longitudinal vertical section through the salt-bath container;

Figure 6 is a diagram illustrating the shearing off of the stud;

Figure 7 is an elevation of the upper end of the billet showing the hook for suspending it and the shield for protecting the supporting stud; and

Figure 8 is a set of curves showing the progress of the heating of both stainless and low-carbon steel billets by my invention.

Referring now in detail to the drawings, a billet or slug 10 of the desired composition and having the size and shape appropriate for the intended extrusion, has a stud 11 of low-carbon steel flash-welded to one end thereof normal to the surface thereof as shown in Figure 1. The billet will usually be a cylinder several inches in diameter having a length two or three times the diameter and weighing several hundred pounds. The stud is preferably headed and its shank has such diameter as to provide a section sufficient to carry the billet suspended thereby without substantial elongation when heated to the maximum billet temperature required for extrusion.

The stud welding may conveniently be effected by a conventional device 12 designed for such purpose and available commercially. This device operates first to strike an electric arc between the stud and billet and then, after fusing a pool of metal in the surface of the latter, to thrust the stud forcibly therewith and hold it there until the molten metal solidifies. Such a weld, when cold, has a strength greater than that of the stud proper. Even at elevated temperatures, say 2300° F., the weld strength is approximately equal to that of the stud. A plurality of studs may be used, depending on the weight to be supported since the latter determines the total sectional area of studs needed for a given billet.

When the stud has been welded to the billet, the latter is hung on a supporting hook 13 depending from a conveyor trolley (not shown). The hook is slotted or bifurcated to receive the shank of the stud and engage the underside of its head. The trolley from which the hook depends travels above a furnace 14 of the panel type having a longitudinal slot in the top thereof through which the shank of the hook passes. The billet is thus quickly heated by burners 15 mounted in the spaced side walls or panels of the furnace, as it travels along the length thereof. While only one billet is shown in the furnace, it will usually be preferable to pass a continuous succession of billets therethrough in close order.

Instead of a headed stud and a bifurcated hook, I may use headless studs and engage them with gripping jaws carried by a traveling trolley.

The firing rate of the burners, the speed of travel of the billets and the length of the furnace are correlated so that the billets are rapidly heated to a temperature of about 2300° F. The total heating time should be not more than about six minutes per inch of diameter of the billet and is preferably less, i. e., from three to five minutes per inch of diameter. By reason of the rapid heating, the studs which will carry the load stated for thirty minutes, may be relied on to suspend the billets safely. The heating of the billets according to the invention is shown graphically in Figure 8 for both stainless steel and carbon steel. As there shown, the latter heats more rapidly at first but, because of the dip in the curve, is soon overtaken by the stainless-steel billet. In both cases, the heating curve is steep and smooth. The heating rate shown far exceeds the maximum rate heretofore thought feasible for stainless steel. An important result of the rapid heating is that only a thin layer of scale is formed on the billets, which is light and flaky in character. Such scale can be easily and thoroughly removed thus saving die wear and insuring a good surface on the finished product.

In order to reduce the loss of strength by the stud supporting the billet as they are both heated during travel through the furnace, I may employ a cylindrical shield 16 of thermal insulation surrounding the stud and resting on the top of the billet, as shown in Figure 7. Such a shield utilizes the so-called "stack effect." That is to say, the ascent of hot gases through the central region of the shield will induce a downflow of cool air along the inner surface of the wall thereof, which keeps the stud at a temperature somewhat lower than that of the billet. In addition, the shield serves as a radiation barrier and the weld as a conduction barrier. The combined effect is aided by the

cooling effect of the hook which keeps the stud several hundred degrees below the temperature of the billet.

The billets may be rotated as they pass through the furnace, if desired, as by rotating the hooks on which they are suspended, for greater uniformity of heating.

On reaching the exit end of the furnace after being heated to a forging temperature of from 1950° to 2300° F., the billets are subjected to a descaling operation as by being lowered into a tank 17 fitted with a plurality of nozzles 18 discharging water sprays at high velocity. Because of the light, flaky character of the scale resulting from the rapid heating of the billets, it is effectively dislodged by such sprays so quickly that no substantial cooling of the billet occurs.

The heated billets are next immersed in an elongated tank 19 containing a bath of fused salt such as barium chloride, heated to a temperature approximating the desired final temperature of the billets, and caused to travel therethrough, thus continuing the immersion for a short time. The salt bath serves several purposes. In the first place, it exerts a descaling action so that the descaling by water sprays may be omitted if desired. The salt bath also equalizes the temperature in various portions of the billet. Finally it forms a film on the surface of the billet which acts as a lubricant during the extrusion. On reaching the exit end of tank 19, the billet is raised therefrom, and suspended over the charging chute 20 leading to the inlet to the extrusion press. Then the stud 11 is cut off by shears 21. The billet is thus immediately delivered to the extrusion press for hot working therein.

It is to be noted that the invention is characterized by numerous advantages some of which have already been mentioned. Outstanding among these is the reduction in the power required by the extrusion press for working billets heated according to the invention. In fact, the extrusion ratio of a given press may thereby be increased by as much as 10 or 15%. Rapid heating is facilitated by the method of supporting the billets on a suspending stud and by the use of a panel-type furnace. The thin scale formed during the quick heating is easily removable and so permits avoidance of the destructive effect thereof on the forming dies. In addition, the yield of product per billet is increased by reducing the amount of scale. By using a suitable conveyor, the billets may be conveyed through the furnace, descaler and salt bath without disengagement from the supporting hooks 13, thus expediting the overall heating cycle and eliminating conveying baskets or carriers which are very expensive and have but a limited life.

Although I have disclosed herein the preferred embodiment of my invention, I intend to cover as well any change or modification therein which may be made without departing from the spirit and scope of the invention.

I claim:

1. In a method of heating billets to temperatures suitable for extrusion, forging or the like, the steps including

providing a billet having a metal suspending attachment welded to one end thereof, engaging the attachment with a traveling support to suspend the billet, then passing the suspended billet and at least a portion of the attachment through an elongated heating chamber, thereby subjecting substantially the entire surface of the suspended billet uniformly to the heat of the chamber and heating the billet at a rate such that it reaches a forging temperature exceeding 2000° F. before the strength of the attachment falls below the weight of the billet.

2. The method defined by claim 1 characterized by shearing said attachment while the billet remains suspended from said support and delivering the billet by gravity to hot-working means.

3. The method defined by claim 1 characterized by said attachment having a head and said support engaging the under side thereof.

4. The method defined by claim 1 characterized by supplying heat to the billet as it traverses the chamber at a rate such as to heat the billet to forging temperature in a time of from three to five minutes per inch of transverse dimension.

5. The method defined by claim 1 characterized by shielding the attachment throughout its entire length while the billet is passing through the chamber.

6. The method defined by claim 1 characterized by descaling the billet as it emerges from the heating chamber and then immersing the billet in a bath of fused salt heated to about the same temperature as the billet.

7. The method defined by claim 1 characterized by subjecting the heated billet to a water-spray descaling as it emerges from the heating chamber.

#### References Cited in the file of this patent

#### UNITED STATES PATENTS

| Number    | Name           | Date           |
|-----------|----------------|----------------|
| 1,382,002 | Leslie et al.  | June 21, 1921  |
| 1,657,580 | Miller         | Jan. 31, 1928  |
| 1,919,136 | Smith          | July 18, 1933  |
| 1,926,770 | Harris et al.  | Sept. 12, 1933 |
| 2,156,008 | Boland         | Apr. 25, 1939  |
| 2,372,478 | Farr et al.    | Mar. 27, 1945  |
| 2,464,163 | Weesner et al. | Mar. 8, 1949   |
| 2,480,516 | Stanier et al. | Aug. 30, 1949  |
| 2,489,459 | Ness et al.    | Nov. 29, 1949  |

#### FOREIGN PATENTS

| Number  | Country | Date          |
|---------|---------|---------------|
| 692,253 | Germany | June 15, 1940 |

#### OTHER REFERENCES

"High Speed Heating of Steel" by Mawhinney in Industrial Heating, January 1951, vol. XVIII, No. 1, pages 40-44, inclusive.